

## UNITED STATES PATENT OFFICE

2,163,067

## RESISTANCE ELEMENT

Newton C. Schellenger, Elkhart, Ind., assignor to  
Chicago, Telephone Supply Co., Elkhart, Ind.,  
a corporation of Indiana

No Drawing. Application December 18, 1935,  
Serial No. 55,005

6 Claims. (Cl. 201—76)

This invention relates to a new and improved resistance element and more particularly to resistance elements comprising ingredients tending to stabilize the resistance value under varying 5 conditions of temperature and moisture.

The invention is particularly directed to resistance elements comprising a high resistance coating on a substantially non-conducting base. These resistances comprise bases of paper, fibre, 10 Bakelite or other artificial resins and conductive coatings consisting of carbon in various forms, with different types of vehicles and binders. These coatings are usually painted or sprayed 15 upon the bases. Some of them harden or cure merely on exposure to the air, while others require varying degrees of heat to drive off volatile constituents and react or cure the binder. In modern radio circuits these resistances are used 20 as tone and volume controls and are included in sensitive portions of the circuits. Design practice has tended to reduce the size of these controls so that the resistance strip is arcuate in form and usually of a diameter of less than one and a half inches. The units are also of a thickness of less 25 than seven-sixteenths of an inch so that, in order to accommodate the contacts, contact arms and other structural elements, the resistance itself must be of slight thickness.

Into these units are placed resistance elements 30 which frequently measure as high as several megohms. In addition, the resistance gradient in nearly all cases must be built to very close progression tolerances and must accurately conform to such irregular curve forms as the radio set engineer may specify for the proper control of a given radio set. For such elements to give commercial service they must be stable under varying 35 operating conditions, particularly with reference to varying degrees of relative humidity.

40 Radio inspection departments often put such units through severe humidity tests and require a high degree of stability of resistance throughout repeated cycles of a wide range of temperature and humidity conditions. Some controls now manufactured will show an increase in resistance above that at normal conditions, which reaches as high as 80% when subjected to a relative humidity of 90% at a temperature of 100° 45 F. over a period of fifty hours. Some of the more stable types of resistance elements show a resistance increase of only from 8% to 20% above normal under similar humidity tests. Even these latter increases above normal are, in the 50 majority of cases, highly detrimental to the func-

tioning of the radio circuit in which they are used.

It is an object of the present invention to provide a new and improved resistance element which is stable under severe changes of temperature and humidity.

It is a further object to provide means whereby various types of resistance elements may be rendered stable under the conditions stated.

It is an additional object to provide methods 10 for making and stabilizing resistance compounds and elements.

It is also an object to provide means, methods and elements of this character which are comparatively low in cost, simple in use and adapted 15 for commercial production.

Other and further objects will appear as the description proceeds.

Broadly my invention comprises the addition to or association with a high resistance element 20 of a constituent which has a lower electrical resistance when it is submitted to conditions of higher humidity than under normal conditions. Since the high resistance element itself has a 25 definite trend toward increase of resistance under conditions of high humidity, the stabilizing constituent by its decrease in resistance under the same conditions may be added in such proportions as to directly counterbalance the trend of the resistance unit and make a combined unit 30 which is extremely stable under such conditions.

I have used a number of different stabilizing agents in combination with various types of resistance compounds and have found that there 35 are many salts and a number of mild acids which may be effectively used for this purpose. Among the salts I have found sodium chloride to be particularly effective. Other neutral salts which may be used include sodium sulphate and ferric chloride, while the basic salts, sodium carbonate and sodium tetraborate, are also suitable, as is the double salt ferric ammonium sulphate. Mild inorganic acids, such as boric or arsenic acids, may be used or organic acids, such as tannic acid. I preferably use sodium chloride as I have found 40 it to be simple and effective in use and it may be readily secured in sufficient purity at low cost.

The sodium chloride may be added to or incorporated with the resistance element in several ways, and the most effective way depends upon 50 the character of the unit with which it is used. I have found that the quantity required is relatively small and generally is somewhere between one-quarter of one percent and four percent of the weight of the conductive pigments being em- 55

ployed. The proper amount for each type or combination of pigments, vehicles and binders must be determined by experiment.

In one method of incorporating the stabilizing agent it is first reduced to a very fine powder in a ball mill. It is then introduced into a second ball mill with the conductive pigments, which comprise finely divided carbon, and the mixture ground in the mill for a period of approximately nine hours. As a binder for the solid constituents in this method, I use pyroxylin or nitrated cotton. This binder has no chemical effect on the stabilizing salt. Other binders which may be used include Bakelite resin, vinyl resin, fufural resin, and other materials of the same general character.

The mixture is sprayed onto the bases to form a thin film and is air dried at moderate temperatures. In some cases sheet Bakelite is used for the bases and in other cases paper approximately .020" in thickness is used. Repeated tests show that the stabilizing effect of the salt is just as permanent in the film on Bakelite as it is when used on the more absorbent paper base or supporting member.

By the use of my stabilizer or neutralizing ingredient in the resistance element, I am able to hold the resistance characteristics within a range of one to two percent when the element is subjected to the most adverse operating conditions, that is, high relative humidity and high temperature. In all cases the element returns to its normal condition when the moisture content is reduced to its original proportions.

With resistance elements of a wholly carbonaceous character, I have found it is not generally desirable to mix the stabilizing material with the pigments and binder before subjecting them to the high temperature used to cure or react the binder. This is not desirable when the necessary temperatures are such as to affect the stabilizing agent and thus impair its later action as a stabilizer. In such cases I have found it desirable to take the salt in solution and spray it upon the surface of the resistor after the resistor has been through its heat treatment. The minute cavities in the surface of the resistance unit hold the salt after the moisture has been driven off. Only a small loss in effectiveness was found in such units after many cycles of high humidity in the testing apparatus.

With some types of resins when used as binders for the resistance particles, such, for example, as vinyl resin, I have found that the surface is not sufficiently porous to effectively hold the stabilizing agent and in such cases the agent may be sprayed upon the base before the resistance material is applied. In such cases the stabilizing agent goes through the heat treatment accorded the unit but is less affected by the heat than if incorporated with the resistance compound.

Thus it will be seen that my stabilizing agent may be used in several ways, depending upon conditions. It may be incorporated with the resistance material or may be applied to the surface of either the resistance carrying base or of the resistance material after the latter has gone through relatively severe heat treatment. While I prefer to use sodium chloride, other agents, such as other salts and certain mild acids, have been found to be suitable. The essential characteristics of the stabilizing agent are that it re-

duce resistance under conditions of high humidity, that it be relatively inert toward the constituents of the resistance element and the contacts, and that it be capable of repeated reversal in going through cycles of humidity without substantial loss in effectiveness.

Since the increase in resistance due to humidity varies with different combinations of resistance materials and binders, the amount and character of the stabilizing material for use with different resistance units will vary and can best be determined by experiment.

While I have disclosed certain preferred embodiments of my invention, these are to be taken as illustrative only, as it is capable of change and variation to meet differing conditions and requirements and I contemplate such modifications as come within the spirit and scope of the appended claims.

I claim:

1. In a resistance element, in combination, carbonaceous resistance material, a resinous binder for said material, the resistance of said material and binder increasing with increases in humidity, and a stabilizing agent associated therewith, said agent having a resistance which decreases with increases of humidity, said increases and decreases in resistance substantially counterbalancing each other.

2. In a resistance element, in combination, carbonaceous resistance material, a stabilizing agent intimately mixed with the resistance material, and a binder for the material and agent, the stabilizing agent being reversely affected as to conductivity by moisture to the effect of moisture on other constituents whereby the resistance value of the combination remains substantially constant through variations in humidity.

3. In a resistance element, in combination, finely divided carbonaceous resistance material, a finely divided stabilizing agent intimately mixed with the resistance material, and a resinous binder for the material and agent, the stabilizing agent being reversely affected as to conductivity by moisture to the effect of moisture on other constituents whereby the resistance value of the combination remains substantially constant through variations in humidity.

4. A resistance element comprising carbonaceous material, sodium chloride, and a binder, the sodium chloride constituting a small percentage of the total and being present in such quantity as to maintain the resistance of the unit substantially constant under fluctuating temperature and humidity conditions.

5. The method of making a substantially stable resistance element, which comprises reducing sodium chloride to a fine powder, adding the sodium chloride to carbonaceous material, adding a binder, treating the mixture to thoroughly mix the sodium chloride and carbonaceous material, and to finely divide them, and placing a thin layer of the mixture on a substantially non-conducting base.

6. The method of making a substantially stable resistance element, which comprises reducing a stabilizing agent to a fine powder, adding the agent to carbonaceous material and a binder, treating the mixture to thoroughly mix and finely divide the materials, and placing a layer of the material on a substantially non-conducting base.

NEWTON C. SCHELLENGER.